

## UNITED STATES PATENT OFFICE

2,514,234

PROCESS FOR THE MANUFACTURE OF  
COLOR PHOTOGRAPHIC IMAGES

Béla Gaspar, Beverly Hills, Calif., assignor to  
Chromogen, Incorporated, a corporation of  
Nevada

No Drawing. Continuation of application Serial  
No. 541,282, June 20, 1944, which is a division  
of application Serial No. 518,256, January 14,  
1944, which in turn is a division of application  
Serial No. 351,907, August 8, 1940. This applica-  
tion October 14, 1947, Serial No. 779,839. In  
Great Britain August 9, 1939

6 Claims. (Cl. 95—88)

1

The present application is a continuation of  
my application Serial No. 541,282, filed June 20,  
1944, now abandoned. Application Serial No.  
541,282 is a division of my application Serial No.  
518,256, filed January 14, 1944, which in turn is  
a division of my Patent 2,361,541 which relates  
to the production of dye images from photo-  
graphic silver images by a process which com-  
prises the synthesis of an azo dye in the exposed  
photographic emulsion layer.

In my prior United States Letters Patent No.  
2,071,688, dated February 23, 1937, I have de-  
scribed and claimed a method of producing color  
photographic images in which the photographic  
layer is subject to two treatments, the first treat-  
ment consisting in the conversion of a dye-form-  
ing substance into a dye and the second treatment  
consisting in the local dye destruction at the re-  
quired points in accordance with my Patent  
2,029,775. Thus, for example, a diazo compound  
is transformed into an azo dye by coupling with  
a phenol; or a phenol or other azo coupler is  
transformed into an azo dye by treating with a  
diazo compound, the azo dyes thus formed then  
being destroyed locally.

In my prior British Patent Specification No.  
416,660, as well as in Patent 2,071,688 just men-  
tioned, I have also described and claimed an  
alternative process in which the first treatment  
consists in the local destruction of the dye-form-  
ing substance, the second treatment then con-  
sisting in the conversion of the remaining dye-  
forming substance into the dye.

If, for carrying out the processes referred to  
above, a layer is used which contains either an  
azo coupler or a diazo compound but not both,  
the production of the dye image can be performed  
either by coupling with a diazo compound or  
coupling with an azo coupler, respectively, and  
the destruction at the image or non-image parts  
of the dye thereby obtained.

If, however, the layer contains a diazotizable  
amino compound and an azo coupler, the process  
includes the step of diazotization, in addition to  
coupling and destruction at the image or non-  
image parts of either the diazo compound or the  
dye.

The present invention relates to the treatment  
of photographic layers that either comprise both  
a diazotizable amino compound and a compound

that is capable of coupling with diazo compounds  
or that comprise a compound which is both  
diazotizable and then capable of coupling with  
itself. The operations of diazotization, coupling  
and destruction at the image parts are not car-  
ried out in three separate treating steps but with  
only two baths or even with one single bath.

This simplification of the process is rendered  
possible by the present invention which consists  
in imparting a triple function to the treating  
solution or a dual function to one of two treating  
solutions so that the same treating solution is  
capable of bringing about diazotization, coupling  
and destruction at the image or non-image parts  
or at least two of these effects. Different pos-  
sibilities of carrying out the invention are illus-  
trated by the following examples.

*Example 1.*—A photographic layer comprising  
a metallic silver image and the substance  
20 (p - aminobenzoyl) - p - amino - benzoyl - 1 -  
amino-8-naphthol-3,6-disulphonic acid



30 which is distributed diffusely throughout the  
layer is treated for about 5 minutes with a solu-  
tion of 250 ccs. of a 0.25-normal sulphuric acid  
and 1 cc. of a 0.1 normal-sodium nitrite solution.  
35 The image is washed and immersed for about  
5 minutes into a 2.5% thiocarbamide solution  
containing 2% acetic acid which causes coupling  
of the diazotized amino compound simultaneously  
with destruction at the points of the silver image.  
40 The silver image is thereafter removed in the  
usual manner by bleaching with cupric chloride  
solution and fixing. A reversed red dye image  
is thus obtained.

*Example 2.*—An image as used in Example 1 is  
45 treated with a solution of 20 ccs. 0.1-normal  
acetic acid with the addition of a 0.1 cc. of a  
0.1-normal sodium nitrite solution. Diazotiza-  
tion and coupling and the formation of an image  
occur within the same solution. After about  
50 10 to 20 minutes the silver is removed from the

dye image. The dye image can be improved by treating the layer prior to the removal of the silver with a dye destroying solution, such as a 5% hydrobromic acid solution.

**Example 3.**—A silver image as used in Example 1 is treated with a solution of 20 ccs.  $\frac{1}{2}$ -normal acetic acid containing 5% sodium chloride and 0.1 cc. of a 0.1-normal sodium nitrite solution. After 20 minutes the silver image is removed by a cupric salt solution and fixing; a dye image is obtained.

**Example 4.**—A silver image as used in Example 1 is treated with 25 ccs. of a solution of 0.25-normal hydrobromic acid to which 0.1 cc. of a 0.1-normal sodium nitrite solution have been added which acts to diazotize and to destroy the diazonium compound at the points of the silver image. The layer is after-treated with a 0.25-normal sodium carbonate to cause the diazotized compound to couple. The silver is removed and a reversed dye image obtained.

From the foregoing examples it will be seen that the triple function of diazotizing, coupling and destruction of the dye or dye-forming substance is given to one single treating solution, or that two of these functions are given to the one of two treating baths employed in the examples. Instead of the coupling component used in the examples, other components may be used; for example, a mixture of a diazotizable amino compound, such as Diazo Light Yellow (described and claimed in my aforementioned Patent 2,071,688 as a compound which fastly dyes a silver halide emulsion), and a coupling compound, such as carbonyl-bis-[8-(4-(4-amino-benzamino)-benzamino)-naphthol-(1)-disulphonic acid-(3,6)] (Beilstein's Handbuch der Organischen Chemi, 4th ed., 1933, Suppl. Vol. XIV, page 759, Formula XI on page 758).



may be used which are distributed diffusely throughout a layer.

The process of the present invention for the production of color photographic images is especially useful for the manufacture of multi-color images in a plurality of layers. In the multi-layer material used for this process some or all of the layers may contain a dye-forming substance capable of coupling with itself or some or all of the layers may contain a diazotizable amino compound and a compound that is capable of coupling with diazo compounds.

I claim:

1. A process for producing a reversed photographic dyestuff image in a layer comprising a silver image and a diazotizable amino compound distributed diffusely throughout said layer, which comprises treating said layer with a solution which causes said compound to be diazotized and then treating said layer with a single solution to produce a reversed dyestuff image which solution causes coupling of the diazotized compound to form a dye in the presence of a substance which is non-destructive with respect to said dye but reacts with said silver image to oxidize it and substantially simultaneously to form a reducing substance.
2. A process for producing a reversed photo-

graphic dyestuff image in a layer comprising a silver image together with a diazotizable amino compound and a compound capable of coupling with diazo compounds, said compounds being uniformly distributed throughout said layer, which comprises treating said layer with a solution which causes diazotizable amino compound to be diazotized and then treating said layer with a single solution to produce a reversed dyestuff image which solution causes coupling of the diazo compound with the compound capable of coupling thereto to form a dye in the presence of a substance which is non-destructive with respect to said dye but reacts with said silver image to oxidize it and substantially simultaneously to form a reducing substance.

3. A process for producing a reversed photographic dyestuff image in a layer comprising a silver image and an amino compound distributed diffusely throughout said layer which is both diazotizable and then capable of coupling with itself to form a dye, which comprises treating said layer with a solution which causes said compound to be diazotized and then treating said layer with a single solution to produce a reversed dyestuff image which solution causes the diazotized compound to couple with itself to form a dye in the presence of a substance which is non-destructive with respect to said dye but reacts with said silver image to oxidize it and substantially simultaneously to form a reducing substance.

4. A process for producing a reversed photographic dyestuff image in an emulsion layer comprising a silver image and a diazotizable amino compound possessing dyeing properties with respect to the emulsion layer distributed diffusely throughout said layer, which comprises treating said layer with a solution which causes said compound to be diazotized and then treating said layer with a single solution to produce a reversed dyestuff image, which solution causes coupling of the diazotized compound to form a dye in the presence of a substance which is non-destructive with respect to said dye but reacts with said silver image to oxidize it and substantially simultaneously to form a reducing substance.

5. A process for producing a reversed photographic dyestuff image in an emulsion layer comprising a silver image together with a diazotizable amino compound possessing dyeing properties with respect to the emulsion layer and a compound capable of coupling with diazo compounds, said compounds being uniformly distributed throughout said layer, which comprises treating said layer with a solution which causes said diazotizable amino compound to be diazotized and then treating said layer with a single solution to produce a reversed dyestuff image, which solution causes coupling of the diazo compound with the compound capable of coupling thereto to form a dye in the presence of a substance which is non-destructive with respect to said dye but reacts with said silver image to oxidize it and substantially simultaneously to form a reducing substance.

6. A process for producing a reversed photographic dyestuff image in a layer comprising a silver image and a diazo compound distributed diffusely throughout said layer, which comprises treating said layer with a single solution to produce a reversed dyestuff image, which solution causes coupling of the diazo compound to form a dye in the presence of a substance which is non-destructive with respect to said dye but reacts

with said silver image to oxidize it and substantially simultaneously to form a reducing substance.

BÉLA GASPAR.

REFERENCES CITED

The following references are of record in the file of this patent:

UNITED STATES PATENTS

| Number    | Name  | Date         |
|-----------|-------|--------------|
| 1,758,572 | Lierg | May 13, 1930 |

| Number      | Name             | Date          |
|-------------|------------------|---------------|
| 2,020,775   | Gaspar           | Nov. 12, 1935 |
| 2,071,688   | Gaspar           | Feb. 23, 1937 |
| 2,333,126   | Schwarc          | Nov. 2, 1943  |
| 5 2,361,541 | Gaspar           | Oct. 31, 1944 |
| 2,376,822   | Schneider et al. | May 22, 1945  |

FOREIGN PATENTS

| Number     | Country       | Date           |
|------------|---------------|----------------|
| 10 298,979 | Great Britain | Feb. 20, 1930  |
| 416,566    | Great Britain | Sept. 10, 1934 |